

## UNITED STATES PATENT OFFICE

2,536,050

## TREATMENT OF CELLULOSIC TEXTILE MATERIALS AND PRODUCTS THEREOF

Linton A. Fluck, Jr., Norwalk, Conn., assignor to  
 American Cyanamid Company, New York,  
 N. Y., a corporation of Maine

No Drawing. Application November 10, 1947,  
 Serial No. 785,188

16 Claims. (Cl. 117—139.4)

1

This invention relates to the treatment of cellulosic textile materials and to the products thereof. More particularly the invention is concerned with the production of cellulosic textiles, specifically cotton fabrics, having improved properties (e. g., better resistance to creasing or wrinkling) by a process which comprises impregnating the textile with a particular combination of impregnants within a definite range of proportions of each. Conditions also are maintained that the amount of combined impregnants which are retained by the textile is kept within definite limits.

Generally described, my process of improving the properties of cotton and other cellulosic textiles comprises impregnating such textiles with a combination of (1) a curable (more particularly heat-curable) product of partial reaction of ingredients comprising melamine and formaldehyde, e. g., dimethylol melamine, trimethylol melamine, the heat-curable or thermosetting alkylated, specifically methylated, methylol melamines, etc., which partial reaction product is at least partly soluble and preferably substantially completely soluble in water, and (2) a film-forming, substantially water-insoluble, thermoplastic product of polymerization of a polymerizable mass including a lower alkyl acrylate, e. g., methyl acrylate, ethyl acrylate, n-propyl acrylate, isopropyl acrylate, n-butyl acrylate, isobutyl acrylate, sec.-butyl acrylate, etc., or mixtures thereof with each other or with other monomers or partial polymers which are copolymerizable therewith to yield film-forming, substantially water-insoluble, thermoplastic copolymers or interpolymers. The products of (1) and (2) should be used in a weight ratio corresponding to form 1 to 3 parts of the latter for each part of the former. After the cellulosic textile material has been impregnated with the aforementioned combination of impregnants in any suitable manner, but preferably by treating the textile material, as by immersion, with a substantially homogeneous aqueous composition containing the mixed impregnants in dispersed or other form, the partial reaction product of (1) is cured in situ in intimate contact with the polymerization product of (2) to a substantially water-insoluble state. The total amount of the products of (1) and (2) that are applied to the cellulosic textile material is such that the finished textile contains from about 8 to about 40%, more particularly from 10 to 30%, by weight of the dry (net dry) textile, of a substantially wash-fast impregnant consisting of the product of (1)

2

in a cured or substantially water-insoluble state and the substantially water-insoluble product of (2).

The treatment of cellulosic textile materials with a water-soluble, curable methylated methylol melamine heretofore has been known and is described, for example, in Patent No. 2,339,203 of Harold W. Stiegler and Linton A. Fluck, Jr., issued January 11, 1944. It was also suggested prior to my invention that textile materials, including cotton textiles, be impregnated with various thermoplastic materials, among which polymers of unsaturated aliphatic aldehydes and polymeric esters of unsaturated aliphatic acids, e. g., polymeric methyl acrylate, specifically have been mentioned. In some cases it has been contended that such thermoplastic materials impart increased resistance to creasing or wrinkling to the textile, but, at least in the case of cotton fabrics or cloths, such contentions are inconsistent with available evidence. In general, a thermoplastic impregnant when applied alone to a cellulosic textile material, specifically a cotton fabric, in amounts such as are employed in practicing my invention merely imparts a permanent non-spring finish to the fabric. There is no substantial improvement, if any, in the resistance of the fabric to creasing or wrinkling, and in many cases the tendency of the treated fabric to crease or wrinkle is even greater than that of the untreated fabric.

When cotton fabrics are impregnated with a water-soluble, curable methylated methylol melamine, e. g., in the form of an aqueous solution, and the treated fabric thereafter dried and heated to cure the impregnant to a substantially water-insoluble condition, the resistance of the fabric to shrinking and creasing is considerably increased. However, the tensile strength of the fabric is materially lowered by this treatment, the percentage loss in tensile strength in some cases being as much as 35% or more of that of the original fabric.

The present invention is a solution to the problem of imparting a higher degree of crease resistance to cotton textiles, and especially to mercerized cotton fabrics, than has been obtained with the prior treating agents and to effect this result while at the same time obviating or minimizing losses in the tensile strength of the treated textile as compared with the untreated material.

The invention involved herein is based on my discovery that cellulosic textile materials, more particularly textiles comprising natural fibers

and specifically cotton fabrics, can be rendered resistant to creasing and the losses in tensile strength either obviated or materially lessened by treating the fabric as briefly described in the first and second paragraphs of this specification and more fully hereafter. In general, the degree of crease resistance imparted to the fabric is greater than that obtained by using only a curable methylated methylol melamine or other curable, water-soluble or -dispersible product of partial reaction of ingredients comprising melamine and formaldehyde. This was wholly unexpected and unpredictable, since the thermoplastic polymerization product alone does not impart marked crease resistance, if any, to a cotton fabric. It also was surprising and unexpected that the thermoplastic polymerization product would obviate or decrease the loss in tensile strength which normally results when a cotton textile is impregnated with a curable methylated methylol melamine, or equivalent curable product of partial reaction of ingredients comprising melamine and formaldehyde, and thereafter dried and cured, since from the known properties of thermoplastic polymers and copolymers it would not be expected that such materials would co-act, physically or otherwise, with the methylated methylol melamine or equivalent material so that the embrittlement of the textile, as evidenced by a decrease in its tensile strength, would be obviated or minimized.

The impregnated cotton and other cellulosic textiles of my invention also are resistant to shrinking, as well as to wear and abrasion. The finish is durable and is not removed by washing in water. The hand may be varied considerably, for example, by varying the kind and amount of thermoplastic modifier employed and by variations in the impregnating and finishing operations. In some cases it may be stiffer than that of fabrics containing a cured methylated methylol melamine alone, which is a characteristic that is desired in many types of cellulosic textiles.

The curable partial reaction products of ingredients comprising melamine and formaldehyde which are used in practicing my invention are at least partly soluble in water, the preferred reaction products being those which are substantially completely soluble therein, either in the form of a true solution or a colloidal dispersion. Examples of melamine reaction products that may be employed are those which comprise one or more polymethylol melamines, more particularly di-, tri-, tetra-, penta- or hexamethylol melamine or mixtures thereof. Such products may be produced in known manner by effecting reaction under neutral or alkaline conditions between melamine and an aqueous solution of formaldehyde in the ratio of 1 mol of the former to from 2 to 6 or more mols of the latter. To avoid the formation of the crystalline material which has lower water-solubility and to obtain the amorphous product of higher water solubility, the mass advantageously is maintained at a temperature not less than about 70° C. during the reaction. In order to minimize polymerization of the monomer, it is usually desirable to keep the reaction temperature from exceeding about 90° C.

The curable, methylated or methyl alcohol-reacted methylol melamines, more particularly methylated polymethylol melamines, are especially suitable for use in practicing my invention. They may be prepared, for example, by effecting reaction under acidic conditions between a polymethylol melamine and methyl alcohol in the

ratio of 1 mol of the former to from 2 to 6 mols of the latter, depending upon the number of methylol groupings in the melamine derivative and the extent of methylation (or etherification) desired. The reaction is stopped before the product becomes hydrophobic, alkali is added in an amount at least sufficient to neutralize the reaction mass, after which the mass is dehydrated under vacuum. Advantageously the methylated methylol melamine, more particularly poly(methoxymethyl) melamine, is prepared in a manner such as is disclosed and claimed in the copending application of Herbert J. West and William T. Watt, Serial No. 568,780, filed December 18, 1944, now Patent No. 2,529,856. Such methylated methylol melamines are miscible with water in all proportions at room temperature and are stable on storage at 120° F. for at least two weeks.

20 The thermoplastic polymerization products are prepared by known methods. Although a polymer of a lower alkyl (e. g., methyl, ethyl, propyl, tert.-butyl, amyl, etc.) ester of acrylic acid may be used as the thermoplastic modifier, I prefer to employ copolymers or interpolymers of such esters (or mixtures thereof) with a suitable proportion of one or more other monomers which are compatible and copolymerizable therewith to yield a water-insoluble, film-forming thermoplastic copolymerization product which is flexible or pliable in film form. Illustrative examples of monomers which may be employed in the production of copolymers useful in practicing my invention are compounds different from the lower alkyl acrylate component and which contain a single  $\text{CH}_2=\text{C}<$  grouping, for instance: the monovinyl compounds (both aliphatic and aromatic), including the vinyl esters of saturated aliphatic monocarboxylic acids (e. g., vinyl acetate, vinyl propionate, vinyl butyrate, etc.); the monovinyl-substituted cyclic compounds, for instance styrene and the various nuclearly substituted styrenes (e. g., the mono- and dimethyl styrenes, the chloro, fluoro and other halogeno styrenes, the cyano styrenes, etc.),  $\alpha$ -p-dimethyl styrene (isopropenyl toluene) and other  $\alpha$ -substituted, nuclearly substituted styrenes, vinyl pyridines, vinyl thiophenes, vinyl fluorenes, etc.; the vinyl and vinylidene halides, e. g., the chlorides, bromides and fluorides; acrylic acid, acrylonitrile and the amides of acrylic acid, e. g. acrylamide and the N-mono- and -di-alkyl acrylamides (e. g., N-methyl acrylamide, N-diethylacrylamide, etc.); alkacrylic compounds, including the acids, esters, nitriles and amides, e. g., methacrylic, ethacrylic, etc., acids, methacrylamide, ethacrylamide, etc., and the N-monoalkyl and -dialkyl substitution products thereof, methacrylonitrile, ethacrylonitrile and other hydrocarbon-substituted acrylonitriles, the methyl, ethyl, propyl, isopropyl, n-butyl, isobutyl, amyl, etc., esters of methacrylic, ethacrylic, etc., acids; the allyl and methallyl esters of saturated monocarboxylic acids, e. g., allyl and methallyl acetates, propionates, laurates, etc.; and numerous other vinyl, vinylidene, acrylic and other compounds containing a single  $\text{CH}_2=\text{C}<$  grouping. In some cases compounds containing a plurality of  $\text{CH}_2=\text{C}<$  groups, e. g., 1,3-butadiene, may comprise the comonomer employed in forming the copolymer. Suitable compounds of this class are those which, like 1,3-butadiene, are compatible and copolymerizable with the lower alkyl acrylate to yield a water-insoluble, film-forming thermoplastic copolymerization product which is flexible or pliable in film form.

It will be understood, of course, by those skilled in the art that the particular monomeric material which is employed in producing the copolymer is so selected and is used in such a proportion with the lower alkyl acrylate, e. g., ethyl acrylate, as to obtain a film-forming material which, when applied to the cellulosic textile in combination with the curable melamine-formaldehyde reaction product, will impart to the treated textile the desired finish and hand.

Particularly good results have been obtained with copolymers of a lower alkyl acrylate, specifically ethyl acrylate, and styrene or acrylonitrile. However, as has been mentioned previously, a polymer instead of a copolymer of a lower alkyl acrylate may be used as the thermoplastic modifier. Thus, I may employ the product of polymerization of a polymerizable mass containing, by weight, from 50 to 100% of a lower alkyl acrylate, specifically ethyl acrylate, and from 50 to 0% of a different monomer which is copolymerizable therewith and which contains a  $\text{CH}_2=\text{C}$  grouping, specifically styrene or acrylonitrile. In some cases the monomeric material which is copolymerized with the monomeric lower alkyl acrylate may constitute as much as 90% by weight of the mixture of monomers, but usually I employ a thermoplastic modifier obtained by polymerization of a mixture containing, by weight, from 70 to 90% of the lower alkyl acrylate and from 30 to 10% of the other copolymerizable monomer. I prefer to use copolymers of, by weight, from 70 to 90% of ethyl acrylate and from 30 to 10% of styrene or acrylonitrile. The polymers and copolymers used in practicing my invention are either substantially water-insoluble per se or yield substantially water-insoluble compositions when the reactive melamine derivative is cured in intimate contact with the polymer or copolymer.

The thermoplastic polymerization products may be prepared in any suitable manner but advantageously are produced by emulsion polymerization (or copolymerization) technique, for example as described in the copending application of Edward L. Kropa, Serial No. 636,279, now abandoned, filed December 20, 1945, with particular reference to the emulsion copolymerization of styrene and certain acrylic esters.

The curable methylated methylol melamine, more particularly methylated polymethylol melamine, or other curable partial reaction product of ingredients comprising melamine and formaldehyde and the thermoplastic polymerization product are ordinarily, and preferably, applied to the cellulosic material in the form of an aqueous dispersion or emulsion containing the aforementioned ingredients, e. g., in a concentration of from 8 to 40%, more particularly from 10 to 30%, by weight thereof. The reactive melamine resin may be in dissolved state and the thermoplastic modifier dispersed in the aqueous solution of the dissolved melamine resin. When the textile is impregnated with 100%, by weight of the dry textile, of the aqueous dispersion, the impregnated textile will contain, after drying and curing of the reactive melamine resin, approximately the same percentage of cured resin admixed with the thermoplastic polymerization product as the percentage of curable melamine resin (or resinifiable material) and thermoplastic additive which is present in the aqueous dispersion. In order to speed up the curing of the curable methylated methylol melamine or other partial reaction product of ingredients comprising melamine and

formaldehyde and to decrease the heating time, a suitable catalyst may be added to the aqueous dispersion, e. g., oxalic acid, acetic acid, phosphoric acid, diammonium hydrogen phosphate, ethyl ammonium phosphate, diammonium phthalate, ammonium chloride, zinc chloride, and others which are known to be catalysts for curing such reaction products. The amount of catalyst may be varied as desired or as conditions may require, but ordinarily the catalyst is employed in an amount corresponding to from 0.5 to 5% by weight of the melamine derivative.

The curable methylated methylol melamine or other melamine derivative of the kinds aforementioned and thermoplastic polymerization product are employed in the ratio of, by weight, 1 part of the former to from 1 to 3 parts (preferably from 1 to 2 parts) of the latter. The thermoplastic modifier must be used in a weight ratio which is at least equal to that of the melamine derivative in order to obtain the results (e. g., better crease resistance, minimizing or obviating tensile strength losses, etc.) hereinbefore set forth. If a weight ratio of thermoplastic modifier to melamine derivative materially above 3 to 1 be employed, the impregnated cloth is excessively weighted, usually has a non-drapey hand and is not satisfactory for use in applications (e. g., in dresses and other clothing) where the weight and feeling to the touch are important. Good results are obtained by using the curable melamine derivative and thermoplastic modifier in a weight ratio of approximately 1 to 1, or with a relatively small excess of the latter, e. g., up to 50% excess by weight of the thermoplastic additive.

The melamine derivative and thermoplastic polymerization product may be applied to the cotton fabric or other cellulosic textile material in various ways. For example, if the curable reaction product and thermoplastic modifier are applied in the form of an aqueous dispersion, the dry or substantially dry cellulosic fabric to be treated may be immersed in the dispersion and then passed through pressure rolls or padders to secure uniform impregnation and a controlled removal of the excess dispersion. The fabric or other textile, however, may be impregnated by other methods, e. g., by spraying or by means of suitable boxes located on a mangle.

The term "aqueous dispersion" as used generally herein with reference to the aqueous composition containing the reactive melamine resin and thermoplastic modifier includes within its meaning aqueous dispersions in which the reactive melamine resin is present either dissolved in the aqueous phase in the form of a true solution or colloidal dispersed in the said phase.

The pick-up of aqueous dispersion by the cotton or other cellulosic material being treated should be adjusted so that the finished textile will contain from 8 to 40%, more particularly from 10 to 30%, by weight of the dry textile, of the cured resin (e. g., cured methylated methylol melamine) admixed with the particular thermoplastic modifier employed in the ratio of, by weight, from 1 to 3 parts (preferably from 1 to 2 parts) of the latter for each part of the former. The amount of aqueous dispersion picked up by the cellulosic textile, that is, the so-called "wet pick-up," may be varied as desired or as conditions may require and may range, for example, from about 40 to about 150% or more by weight of the dry textile depending, for example, upon the particular textile treated, method and conditions of treatment, concentration of solids in

the impregnating bath, amount of solids and properties desired in the finished textile, etc.

The wet, impregnated cotton fabric or other cellulosic textile material is then dried and cured. The drying and curing temperatures may be varied considerably, but ordinarily temperatures within the range of about 200° F. to about 400° F. are employed. The impregnated fabric may be dried at a relatively low temperature of the order of 200° F. to 212° F. to remove all or most of the water, after which the dried material is heated at a temperature within the range of 250° F. to 400° F. to convert or cure the curable methylated methylol melamine (or equivalent material employed) admixed with the thermoplastic polymerization product, e. g., polymeric ethyl acrylate, a copolymer of ethyl acrylate and styrene or acrylonitrile, etc., to a substantially water-insoluble condition. The drying and curing operation is flexible and may be varied to suit the available equipment. Continuous methods are preferred. However, drying and curing also may be effected by framing the impregnated fabric to width, as on a pin tenter, drying the framed fabric, batching it upon a shell and then allowing it to stand hot for a period sufficient to complete the drying (if not entirely dried previously) and to convert the solid impregnant in situ to a water-insoluble state. In some cases drying and curing for 2 or 3 hours at 200° F. may be required. Heating the dried fabric for 1 minute at 340° F. or for a shorter time at a higher temperature has effectively water-insolubilized the impregnant.

The finishing treatment usually consists in washing the treated textile, e. g., in an aqueous 150°-190° F. solution containing, by weight, from 0.1 to 0.2% of soap and 0.1% soda ash, followed by rinsing in hot water at the same temperature, drying and then calendering either hot or cold.

The process of the present invention may be used in treating both uncolored and colored goods. It is applicable to the treatment of both bleached and unbleached cotton goods, as well as mercerized cotton fabrics. Surprisingly, the results are generally better, especially in plant operations, on mercerized, more particularly scoured and mercerized or bleached and mercerized, materials than on unmercerized cotton textiles.

In order that those skilled in the art better may understand how the present invention may be carried into effect, the following examples are given by way of illustration and not by way of limitation. All parts and percentages are by weight.

The methylated methylol melamine used in all of the examples was a substantially completely water-soluble, heat-curable or thermosetting methylated polymethylol melamine. This material is prepared by the following process: One mol of melamine is mixed with 3.3 mols of aqueous 37% formaldehyde previously adjusted to a pH of approximately 8.0, the temperature being raised to 70° C. and maintained at this point until a clear solution is obtained. The solution is then immediately cooled and allowed to set, after which the mass is broken into small pieces and dried by circulating warm air at a temperature not exceeding 55° C. The resulting dried powder is alkylated by admixture with twice its weight of 95% methanol containing 0.5% of oxalic acid crystals, based on the weight of the methylol melamine. The mixture is heated to 70° C. and held at this temperature for approxi-

mately 15 minutes, or until a clear solution is obtained, whereupon it is immediately neutralized by the addition of sufficient sodium hydroxide solution to raise the pH to approximately 9.0. The neutralized reaction mass is then evaporated to 80% solids under reduced pressure so that the temperature does not rise above 50° C.

#### EXAMPLE 1

In this example the impregnating bath contained 30% of resin solids (10% of methylated methylol melamine plus 20% of a thermoplastic polymerization product) and 0.35% of a curing accelerator, specifically a mixture of diammonium hydrogen phosphate (curing catalyst) and hexamethylene tetramine (buffering agent) in the ratio of about 30 parts of the former to about 4 parts of the latter. The bath was made by diluting with water a composition comprising about 80% methylated methylol melamine and 20% water, and the resulting product was then stirred into an emulsion of the polymerization product.

Impregnation was carried out by soaking the fabric material for about 1/2 minute in the bath and squeezing the impregnated fabric through a padder so that the amount of liquid impregnant retained by the fabric (so-called "wet pick-up") was about 90% by weight of the dry fabric. The squeezed fabric was then heated for 6 minutes at 290° F. to dry the fabric and to cure the applied resinous composition, that is, curable methylated methylol melamine admixed with the particular polymerization product employed, to a substantially water-insoluble state.

The dried textile was then given a mild washing for 2 minutes in an aqueous 160° F. solution containing 0.1% soap and 0.1% sodium bicarbonate, followed by thorough rinsing in water at 160° F. and squeezing of the rinsed fabric. The rinsed and squeezed fabric was then pressed dry on a flat bed electric press.

The fabrics employed in this example were 80 x 80 cotton percale and mercerized cotton twill. The bath compositions each contained 30% by weight of solids, of which 10% of the bath composition was methylated methylol melamine and 20% was a thermoplastic polymerization product. For purpose of comparison a bath containing 10% by weight of methylated methylol melamine and no thermoplastic additive was included in the series of tests. The wet pick-up was about 90% by weight of the dry fabric. The finished fabric contained about 27%, by weight of the dry fabric, of solid, resinous impregnant of which 1/3 was cured methylated methylol melamine resin and 2/3 was thermoplastic modifier. Tables I and II show the thermoplastic materials employed and test data on the treated and lightly washed fabrics. For purpose of comparison data also are given on the untreated fabrics. In these tables and in others which follow "W" means "warp" and "F" means "filling." The total tensile strength (warp plus filling in pounds) is determined using the apparatus and method of the American Society for Testing Materials described under D-76-45.

"Total T. B. L. Crease Resistance (W plus F in cm.)" in the tables refers to the total values of crease resistance of samples of the treated fabrics cut along the warp and along the weft, using the apparatus and procedure developed by Tootal Broadhurst Lee Company, Ltd. (Manchester, England) and described in publications of this company. In this test, strips of fabric

are cut accurately warp-way 4 cm. x 1 cm. and weft-way 1 cm. x 4 cm. Each strip is folded in half and placed under a 500 gram weight, the cross section of which is the same as that of the doubled fabric. After remaining under the weight for 5 minutes, the specimen is hung over a fine wire for 3 minutes. At the end of this time the distance between the ends of the sample is measured by means of a calibrated plane mirror mounted directly below the sample. The

### EXAMPLE 2

Same as Example 1 with the exception that the bath contained 22½% solids (7½% methylated methylol melamine plus 15% of the thermoplastic modifier). The wet pick-up was about 90% by weight of the dry cloth. Table III shows the thermoplastic materials employed and test data on the treated and lightly washed fabrics.

*Table III.—80 x 80 cotton percale—7½% methylated methylol melamine and 15% thermoplastic modifier*

| Test No.                  | Thermoplastic Additive                                 | Total Tensile Strength (W+F in lbs.) | Tensile Loss Due to Treatment (Approx. Percent) | Total T. B. L. Crease Resistance (W plus F in cm.) |
|---------------------------|--------------------------------------------------------|--------------------------------------|-------------------------------------------------|----------------------------------------------------|
| Untreated cotton percale. |                                                        | 91                                   | —                                               | 3.6                                                |
| 10.                       | None                                                   | 68                                   | 25                                              | 5.4                                                |
| 11.                       | Copolymer of 80% ethyl acrylate and 20% styrene        | 82                                   | 10                                              | 6.0                                                |
| 12.                       | Copolymer of 80% ethyl acrylate and 20% acrylonitrile. | 88                                   | 3                                               | 6.5                                                |

ror mounted directly below the sample. The T. B. L. crease-resistance rating is the distance in centimeters between the ends of the sample after it has been subjected to the treatment described above. The total T. B. L. crease-resistance values reported in the tables are in each case the sum of the values obtained upon testing a strip of the fabric cut along the warp and another strip cut along the weft or filling.

30

35

### EXAMPLE 3

Same as Example 1 with the exception that the bath contained 15% solids (5% methylated methylol melamine plus 10% of the thermoplastic modifier). The wet pick-up was about 90% by weight of the dry cloth. Table IV shows the thermoplastic modifiers employed and test data on the treated and lightly washed fabrics.

*Table I.—80 x 80 cotton percale—10% methylated methylol melamine and 20% thermoplastic modifier*

| Test No.                  | Thermoplastic Additive                                    | Total Tensile Strength (W+F in lbs.) | Tensile Loss Due to Treatment (Approx. percent) | Total T. B. L. Crease Resistance (W plus F in cm.) |
|---------------------------|-----------------------------------------------------------|--------------------------------------|-------------------------------------------------|----------------------------------------------------|
| Untreated cotton percale. |                                                           | 91                                   | —                                               | 3.6                                                |
| 1.                        | None                                                      | 69                                   | 24                                              | 5.5                                                |
| 2.                        | Copolymer of 70% ethyl acrylate and 30% styrene           | 89                                   | 2                                               | 5.7                                                |
| 3.                        | Copolymer of 90% ethyl acrylate and 10% acrylonitrile.    | 84                                   | 8                                               | 6.4                                                |
| 4.                        | Copolymer of 80% ethyl acrylate and 20% acrylonitrile.    | 84                                   | 8                                               | 6.9                                                |
| 5.                        | Copolymer of 70% ethyl acrylate and 30% acrylonitrile.    | 84                                   | 8                                               | 6.0                                                |
| 6.                        | Copolymer of 79% ethyl acrylate and 21% dimethyl styrene. | 88                                   | 3                                               | 6.0                                                |

*Table II.—Mercerized cotton twill—10% methylated methylol melamine and 20% thermoplastic modifier*

| Test No.                           | Thermoplastic Additive                           | Total Tensile Strength (W+F in lbs.) | Tensile Loss Due to Treatment (Approx. Percent) | Total T. B. L. Crease Resistance (W plus F in cm.) |
|------------------------------------|--------------------------------------------------|--------------------------------------|-------------------------------------------------|----------------------------------------------------|
| Untreated mercerized cotton twill. |                                                  | 192                                  | —                                               | 4.2                                                |
| 7.                                 | None                                             | 153                                  | 20                                              | 6.1                                                |
| 8.                                 | Polymeric ethyl acrylate                         | 174                                  | 9                                               | 6.4                                                |
| 9.                                 | Copolymer of 80% ethyl acrylate and 20% styrene. | 177                                  | 8                                               | 6.4                                                |

Table IV.—Mercerized cotton twill—5% methylated methylol melamine and 10% thermoplastic modifier

| Test No.                           | Thermoplastic Additive                                 | Total Tensile Strength (W+F in lbs.) | Tensile Loss or Gain Due to Treatment (Approx. Percent) | Total T. B. L. Crease Resistance (W plus F in cm.) |
|------------------------------------|--------------------------------------------------------|--------------------------------------|---------------------------------------------------------|----------------------------------------------------|
| Untreated mercerized cotton twill. | None.                                                  | 192                                  | —                                                       | 4.2                                                |
| 13.                                | None.                                                  | 166                                  | 14                                                      | 5.4                                                |
| 14.                                | Polymeric ethyl acrylate                               | 194                                  | 11                                                      | 5.9                                                |
| 15.                                | Copolymer of 90% ethyl acrylate and 10% styrene.       | 178                                  | 7                                                       | 6.1                                                |
| 16.                                | Copolymer of 90% ethyl acrylate and 10% acrylonitrile. | 188                                  | 2                                                       | 5.8                                                |

<sup>1</sup> Gain.

## EXAMPLE 4

Same as Example 1 with the exception that impregnating baths comprising, by weight, 10% of methylated methylol melamine and 10%, 15%, 20% and 25% of a copolymer of 80% ethyl acrylate and 20% acrylonitrile were used in treating samples of 80 x 80 cotton percale. In addition to the light wash of 2 minutes described in Example 1, the treated samples also were given a 1-hour wash using the same soap solution and procedure except for the difference in time. The resin solids in the various baths are shown in Table V. The wet pick-up was about 90% by weight of the dry cloth.

Table V.—Resin solids bath

| Test No. | Methylated Methylol Melamine, Per Cent | Thermoplastic Additive |                                                        |
|----------|----------------------------------------|------------------------|--------------------------------------------------------|
|          |                                        | Per Cent               | Description                                            |
| 17.      | 10                                     | None.                  |                                                        |
| 18.      | 10                                     | 10                     | Copolymer of 80% ethyl acrylate and 20% acrylonitrile. |
| 19.      | 10                                     | 15                     | Do.                                                    |
| 20.      | 10                                     | 20                     | Do.                                                    |
| 21.      | 10                                     | 25                     | Do.                                                    |

Table VI shows test data obtained on the treated and washed samples. For purpose of comparison data also were given on the untreated cotton percale.

Table VI

| Test No.                          | Total Tensile Strength (W plus F in lbs.) |            | Total T. B. L. Crease Resistance (W plus F in cm.) |            |
|-----------------------------------|-------------------------------------------|------------|----------------------------------------------------|------------|
|                                   | Light Wash                                | 1 Hr. Wash | Light Wash                                         | 1 Hr. Wash |
| Untreated 80 x 80 cotton percale. | 93                                        | 94         | 3.2                                                | 3.3        |
| 17.                               | 65                                        | 67         | 5.9                                                | 6.0        |
| 18.                               | 79                                        | 74         | 6.4                                                | 6.5        |
| 19.                               | 83                                        | 78         | 6.5                                                | 6.6        |
| 20.                               | 86                                        | 86         | 6.4                                                | 6.5        |
| 21.                               | 88                                        | 86         | 6.4                                                | 6.4        |

In all the foregoing examples each of the baths also contained a curing accelerator of the kind and in the percentage mentioned under Example 1.

When the thermoplastic modifiers mentioned in Tables I to IV, inclusive, are employed alone in treating cotton percale or mercerized cotton twill, that is, in the absence of methylated methylol melamine but with other conditions the same as when the methylated methylol melamine alone or with the thermoplastic modifier is used, the total T. B. L. crease resistance of the impregnated

fabric is approximately the same as that of the untreated fabric.

## EXAMPLE 5

Same as Example 1 with the exception that impregnating baths comprising, by weight, 10% of methylated methylol melamine and 10%, 15% and 20% of a copolymer of 90% ethyl acrylate and 10% of styrene were used in treating samples of 136 x 60 mercerized cotton broadcloth. For purpose of comparison samples also were treated by immersion in baths containing, by weight, 10% of methylated methylol melamine (with no copolymer present), and 10%, 15% and 20% of the same copolymer (with no methylated methylol melamine present). The baths containing methylated methylol melamine also contained a curing accelerator of the kind and in the percentage mentioned under Example 1. The resin solids in the various baths are shown in Table VII.

Table VII.—Resin solids in bath

| Test No. | Methylated Methylol Melamine, Per Cent | Thermoplastic Additive |                                                  |
|----------|----------------------------------------|------------------------|--------------------------------------------------|
|          |                                        | Per Cent               | Description                                      |
| 22.      | 10                                     | None.                  |                                                  |
| 23.      | None                                   | 10                     | Copolymer of 90% ethyl acrylate and 10% styrene. |
| 24.      | None                                   | 15                     | Do.                                              |
| 25.      | None                                   | 20                     | Do.                                              |
| 26.      | 10                                     | 10                     | Do.                                              |
| 27.      | 10                                     | 15                     | Do.                                              |
| 28.      | 10                                     | 20                     | Do.                                              |

Table VIII shows test data obtained on the treated and washed samples. For purpose of comparison data also are given on a sample of the untreated mercerized broadcloth which had been immersed in water and dried prior to testing for tensile strength and crease resistance.

Table VIII

| Test No.                                                         | Total Tensile Strength (W plus F in lbs.) | Total T. B. L. Crease Resistance (W plus F in cm.) |
|------------------------------------------------------------------|-------------------------------------------|----------------------------------------------------|
| Untreated 136 x 60 mercerized cotton broadcloth (wet and dried). | 126                                       | 3.2                                                |
| 22.                                                              | 87                                        | 5.2                                                |
| 23.                                                              | 122                                       | 3.6                                                |
| 24.                                                              | 128                                       | 3.4                                                |
| 25.                                                              | 129                                       | 3.6                                                |
| 26.                                                              | 101                                       | 6.1                                                |
| 27.                                                              | 108                                       | 6.0                                                |
| 28.                                                              | 107                                       | 5.9                                                |

From the results of the above tests it will be noted that the combination of the thermoplastic copolymer and methylated methylol melamine

provides a treated cloth having a materially improved crease resistance as compared with the untreated cloth and much better than that shown by cloths which have been treated with the methylated methylol melamine alone or with various percentages of the thermoplastic copolymer alone. Furthermore, the combination of treating agents yields a treated cloth having a higher tensile strength than that obtained by using methylated methylol melamine alone.

Similar results are obtained when other copolymers, e. g., copolymers of, by weight, 70-85% ethyl acrylate and 30-15% styrene, copolymers of, by weight, 70-90% ethyl acrylate and 30-10% acrylonitrile, etc., are substituted for the particular ethyl acrylate-styrene copolymer employed in the above illustrative example.

#### EXAMPLE 6

|                                                                            | Pounds                         |
|----------------------------------------------------------------------------|--------------------------------|
| Aqueous methylated methylol melamine (80% solids)                          | 70                             |
| Emulsion of a copolymer of 90% ethyl acrylate and 10% styrene (25% solids) | 300                            |
| Curing accelerator as in Example 1                                         | 2                              |
| Water                                                                      | Sufficient to make 100 gallons |

The above ingredients were mixed to yield an impregnating bath which had a pH of 7.0. This bath was used in a plant run in treating four different cellulosic fabric materials. The dry fabrics were passed continuously at 48 yards per minute through the bath (2 dips and 2 nips), the bath temperature being 80° F. The impregnated fabrics were dried in a pre-drier at 220° F. and then in a tenter frame at 300° F., followed by heating for 1 minute at 340° F. to cure the methylated methylol melamine admixed with the ethyl acrylate-styrene copolymer to a substantially water-insoluble state. The fabrics were washed in 190° F. water containing 0.2% soap and 0.1% sodium carbonate, followed by rinsing in clear water at 190° F. All but a cotton cord fabric (cloth No. 4) were finished by drying and cold calendering. The wet pick-up of the cloths averaged 75% of the dry weight of the individual cloth. The amount of resin (cured methylated methylol melamine plus copolymer) on the goods (after drying and curing) averaged about 11.8% by weight of the dried fabric, of which about 5% was cured methylated methylol melamine and the remainder ethyl acrylate-styrene copolymer.

A description of the goods treated and the results obtained are given in Table IX.

Table IX

|                                                                        | Cloth No. 1              | Cloth No. 2              | Cloth No. 3                          | Cloth No. 4                      |
|------------------------------------------------------------------------|--------------------------|--------------------------|--------------------------------------|----------------------------------|
| Quantity treated.                                                      | 200 yds.                 | 200 yds.                 | 200 yds.                             | 350 yds.                         |
| Description and properties of cloths.                                  | Bleached and mercerized. | Bleached and mercerized. | Bleached and mercerized, 3-ply cord. |                                  |
| Color.                                                                 | Stripes.                 | Stripes.                 | Stripes.                             | Brown and white. Blue and white. |
| Warp.                                                                  | 100% cotton.             | 100% cotton.             | 100% cotton.                         | 100% cotton.                     |
| Filling.                                                               | do.                      | do.                      | do.                                  | do.                              |
| Per cent shrinkage of untreated cloths.                                | 6.80                     | 5.60                     | 11.39                                | 4.5                              |
| Per cent shrinkage of treated cloths.                                  | 2.0                      | 1.5                      | 3.0                                  | 1.5                              |
| Tensile strength (in lbs.) of untreated cloths (warp x filling).       | 65 x 43.4                | 66.4 x 25.8              | 60 x 29                              | 74 x 62.2                        |
| Tensile strength (in lbs.) of treated cloths (warp x filling).         | 66.2 x 42.4              | 69.2 x 25.0              | 60.0 x 32.8                          | 77 x 63.5                        |
| Total T. B. L. crease resistance of untreated cloths (W plus F in cm.) | 5.2                      | 4.8                      | 5.3                                  | 6.0                              |
| Total T. B. L. crease resistance of treated cloths (W plus F in cm.)   | 6.3                      | 6.2                      | 6.5                                  | 6.9                              |
| Hand and finish of treated cloths.                                     | Good.                    | Good.                    | Good.                                | Very good.                       |

Although I have described my invention hereinbefore with particular reference to the treatment of cotton, specifically cotton fabrics, the

treatment herein described also may be applied to other textiles which are composed substantially or mainly of cellulose or regenerated celluloses, e. g., linen, hemp, jute, ramie, sisal, cellulose acetate rayons, cellulose acetate-butyrate rayons, saponified acetate rayons, viscose rayons, cuprammonium rayons, ethyl cellulose, etc., and mixtures thereof with each other or with cotton. The invention is particularly applicable to the treatment of cotton fabric material, specifically mercerized cotton cloth, and hence such textiles are preferred for treating to improve their properties as hereinbefore described.

Thermoplastic polymerization products other than those comprising polymers and copolymers of lower alkyl acrylates may be combined with a curable methylated methylol melamine or other curable product of partial reaction of ingredients comprising melamine and formaldehyde and the resulting combination or admixture may be used in treating cotton or other cellulosic textile materials in a manner similar to that hereinbefore set forth. Examples of such polymerization products are the polymers (or copolymers) obtained by polymerizing, alone or admixed with each other or with other monomers, the monomeric materials hereinbefore mentioned with particular reference to compounds that may be copolymerized with a lower alkyl acrylate to yield copolymers suitable for use in practicing the present invention. Such polymers and copolymers, however, are not equivalent, in the relationship in which they are used, to the polymers and copolymers of the lower alkyl acrylates.

The terms "textile" and "textile material" as used generally herein and in the appended claims include within their meaning filaments, fibers, threads, yarns, twisted yarns, etc., as such or in woven, felted or otherwise formed fabrics, sheets, cloths and the like.

I claim:

1. The process of improving the properties of a cellulosic textile material which comprises impregnating the said textile material with a combination of (1) a curable product of partial reaction of ingredients comprising melamine and formaldehyde, said product being at least partly soluble in water, and (2) a film-forming substance consisting essentially of a substantially water-insoluble, thermoplastic product of polymerization of polymerizable monomers, said polymerizable monomers consisting of, by weight, from 50% to 100% of a lower alkyl acrylate and up to 50% of a different monomeric compound containing

a  $\text{CH}_2=\text{C}<$  grouping and which is copolymerizable with said acrylate, the products of (1) and (2) being employed in a weight ratio corre-

sponding to from 1 to 3 parts of the latter for each part of the former, and curing in situ the partial reaction product of (1) in intimate contact with the polymerization product of (2) to a substantially water-insoluble state, the amount of the products of (1) and (2) applied to the said textile material being such that the finished textile contains from 8 to 40%, by weight of the dry textile, of a substantially washfast impregnant consisting of the product of (1) in cured state and 10 the product of (2).

2. A process as in claim 1 which includes the additional steps of washing the treated textile material in an aqueous soap-containing solution followed by rinsing in water; drying the washed and 15 rinsed textile; and calendering the dried textile.

3. A process as in claim 1 wherein ethyl acrylate is the lower alkyl acrylate.

4. A process as in claim 1 wherein the component of (2) is a thermoplastic product of polymerization of a mixture of monomers of which not less than 50% by weight thereof is ethyl acrylate and the remainder styrene.

5. A process as in claim 1 wherein the component of (2) is a thermoplastic product of polymerization of a mixture of monomers of which not less than 50% by weight thereof is ethyl acrylate and the remainder acrylonitrile.

6. The process of rendering cotton fabric material resistant to creasing which comprises impregnating said fabric material with from 10 to 30%, by weight of the dry fabric, of a mixture comprising (1) a curable methylated methylol melamine and (2) a film-forming substance consisting essentially of a substantially water-insoluble, thermoplastic product of polymerization of polymerizable monomers consisting of, by weight, from 50 to 100% of ethyl acrylate and up to 50% of styrene, the components of (1) and (2) being present in the said mixture in a weight ratio corresponding to from 1 to 3 parts of the latter for each part of the former, and the said mixture being applied to the said fabric material in the form of a substantially homogeneous aqueous composition containing the same, and thereafter drying the impregnated fabric material and curing the methylated methylol melamine in the presence of the said polymerization product to a substantially water-insoluble state, thereby obtaining an impregnated cotton fabric material containing a substantially washfast solid impregnant and which has a higher tensile strength and a better crease resistance than the same cotton fabric material which has been similarly impregnated with an aqueous composition containing the same amount of the methylated methylol melamine of (1) but none of the thermoplastic material of (2) and thereafter has been similarly dried and cured.

7. A process as in claim 6 wherein the film-forming substance of (2) is a copolymer of monomers consisting of, by weight, from about 70% to about 90% of ethyl acrylate and from about 30% to about 10% of styrene.

8. A process as in claim 6 wherein the methylated methylol melamine of (1) and the film-forming substance of (2) are present in the aqueous composition in a weight ratio corresponding to from 1 to 2 parts of the latter for each part of the former, and the thermoplastic material of (2) is a copolymer of monomers consisting of, by weight, about 90% ethyl acrylate and about 10% styrene.

9. A process as in claim 6 wherein the cotton fabric material is a mercerized cotton cloth.

10. The process of rendering cellulosic fabric material resistant to creasing which comprises impregnating said fabric material with from 10 to 30%, by weight of the dry fabric, of a mixture comprising (1) a water-soluble methylated methylol melamine and (2) a thermoplastic material which is a copolymer of monomers consisting of by weight, from about 70% to about 90% of ethyl acrylate and from about 30% to about 10% of styrene, the components of (1) and (2) being present in the said mixture in a weight ratio corresponding to from 1 to 2 parts of the latter for each part of the former, and the said mixture being applied to the said fabric material in the form of a substantially homogeneous aqueous composition containing the same, drying the impregnated fabric material and thereafter heating the dried material at a temperature within the range of 250° F. to 400° F. to convert the said methylated methylol melamine admixed with the said copolymer to a substantially water-insoluble condition.

11. A cellulosic textile material which is resistant to creasing and which contains from 8 to 40%, by weight of the dry textile material, of a combination of (1) a substantially water-insoluble, cured product which, prior to curing, is a curable product of partial reaction of ingredients comprising melamine and formaldehyde, said 25 curable product being at least partly soluble in water, and (2) a film-forming substance consisting essentially of a substantially water-insoluble product of polymerization of polymerizable monomers, said polymerizable monomers consisting of, by weight, from 50% to 100% of a lower alkyl acrylate and up to 50% of a different monomeric compound containing a  $\text{CH}_2=\text{C}<$  grouping and which is copolymerizable with said acrylate, the said polymerization product being present in the combination thereof with the said curable product, before curing of the latter, in a weight ratio corresponding to from 1 to 3 parts of the former for each part of the latter.

12. A cotton fabric material which is resistant to creasing and which contains from 10 to 30%, by weight of the dry fabric material, of a combination of (1) a substantially water-insoluble, cured product which, prior to curing, is a curable methylated methylol melamine and (2) a film-forming substance consisting essentially of a substantially water-insoluble, thermoplastic product of polymerization of polymerizable monomers, said polymerizable monomers consisting of, by weight, from 50 to 100% of ethyl acrylate and up to 50% of styrene, the said polymerization product being present in the combination thereof with the said curable methylated methylol melamine, before curing of the latter, in a weight ratio corresponding to from 1 to 3 parts thereof for each 55 part of the said curable methylated methylol melamine, and the said cotton fabric material having a higher tensile strength and a better crease resistance than the same cotton fabric material which has been similarly impregnated with the same amount of the same product of (1) but none of the thermoplastic material of (2).

13. A cellulosic fabric material which is resistant to creasing and which is impregnated with from 10 to 30%, by weight of the dry fabric material, of a combination of (1) a substantially water-insoluble, cured product which, prior to curing, is a water-soluble, curable methylated methylol melamine and (2) a thermoplastic material which is a copolymer of monomers consisting of, by weight, from about 70% to about 90%

17

of ethyl acrylate and from about 30% to about 10% of styrene, the said copolymer being present in the combination thereof with the said curable methylated methylol melamine, before curing of the latter, in a weight ratio corresponding to from 1 to 2 parts thereof for each part of the said curable methylated methylol melamine, and the said cellulosic fabric material having a higher tensile strength and a better crease resistance than the same cellulosic fabric material which has been similarly impregnated with the same amount of the same product of (1) but none of the thermoplastic material of (2).

14. A cellulosic fabric material which is resistant to creasing and which is impregnated with from about 10% to about 30%, by weight of the dry fabric material, of a combination of (1) a substantially water-insoluble, cured product which, prior to curing, is a water-soluble, curable methylated methylol melamine and (2) a copolymer of 90% ethyl acrylate and 10% styrene, the said copolymer being present in the combination thereof with the said curable methylol melamine, before curing of the latter, in a weight ratio corresponding to from 1 to 2 parts thereof for each part of the said curable methylated methylol melamine, and the said cellulosic fabric material having a higher tensile strength and a better crease resistance than the same cellulosic fabric material which has been similarly impregnated with the same amount of the same product of (1) but none of the copolymer of (2).

15. The method of rendering a cotton-containing fabric material resistant to shrinking and otherwise improving its properties which comprises immersing the material to be treated in an impregnating bath maintained at a temperature of about 80° F., said bath having a pH of about 7 and being constituted of

**Aqueous methylated methylol melamine (80% solids)** ----- 70

18

**Emulsion of a copolymer of 90% ethyl acrylate and 10% styrene (25% solids) ----- 300**  
**Curing accelerator consisting essentially of a mixture of diammonium hydrogen phosphate (curing catalyst) and hexamethylene tetramine (buffering agent) in the ratio of about 30 parts of the former to about 4 parts of the latter----- 2**

Water Sufficient to make 100 gallons

10 adjusting the wet pick-up of the fabric so that the amount of cured methylated methylol melamine plus the aforementioned copolymer of ethyl acrylate and styrene on the fabric (after drying and curing) averages about 11.8% by weight  
15 of the dried fabric, of which about 5% is cured methylated methylol melamine and the remainder ethyl acrylate-styrene copolymer; drying the wet impregnated fabric at a temperature up to 300° F. followed by further heating at a temperature of 340° F. for a brief period to advance the cure of the methylated methylol melamine in situ to a substantially water-insoluble state; washing the resulting fabric in an aqueous soap-containing solution followed by rinsing in water;  
20 and drying the washed and rinsed fabric.  
25

16. A method as in claim 15 which includes the additional step of cold calendering the dried fabric.

LINTON A. FLUCK, JR.

#### REFERENCES CITED

The following references are of record in the file of this patent:

UNITED STATES PATENTS

| Number    | Name         | Date          |
|-----------|--------------|---------------|
| 2,187,383 | Ludwig       | Jan. 16, 1940 |
| 2,339,203 | Stiegler     | Jan. 11, 1944 |
| 2,378,365 | Swain et al. | June 12, 1945 |
| 2,499,653 | Kropa        | Mar. 7, 1950  |

**Certificate of Correction**

January 2, 1951

Patent No. 2,536,050

LINTON A. FLUCK, JR.

It is hereby certified that error appears in the printed specification of the above numbered patent requiring correction as follows:

Column 1, line 38, for the word "form" read *from*; column 2, line 26, for "non-spring" read *non-springy*; column 4, line 37, for "armomatic" read *aromatic*; column 6, line 57, for "colloidal" read *colloidally*; column 11, line 47, for "were" read *are*; line 64, after "all" insert *of*; column 16, line 3, for "impergnating" read *impregnating*; line 73, for "methyl" read *methylol*;

and that the said Letters Patent should be read as corrected above, so that the same may conform to the record of the case in the Patent Office.

Signed and sealed this 27th day of March, A. D. 1951.

[SEAL]

THOMAS F. MURPHY,  
*Assistant Commissioner of Patents.*